

## UNITED STATES PATENT OFFICE.

STANLEY APGAR AND GEORGE R. HANKS, OF HIGH BRIDGE, NEW JERSEY, ASSIGNORS TO TAYLOR-WHARTON IRON AND STEEL COMPANY, OF HIGH BRIDGE, NEW JERSEY, A CORPORATION OF NEW JERSEY.

## TREATMENT OF MANGANESE-STEEL CASTINGS.

No Drawing.

Application filed June 5, 1922. Serial No. 566,139.

*To all whom it may concern:*

Be it known that we, STANLEY APGAR and GEORGE R. HANKS, citizens of the United States, residing at High Bridge, in the 5 county of Hunterdon and State of New Jersey, have invented certain new and useful Improvements in the Treatment of Manganese-Steel Castings, of which the following is a specification.

10 The object of our invention is to provide a dependable method of heat treating manganese steel castings of large size and intricate section.

We are aware of the method proposed by 15 Brinton in his patent 812,811, and also of the Hadfield method. Brinton's method was undoubtedly an advance over the Hadfield practice, and he refers to the successful heat treatment of castings weighing up 20 to eight tons. But present day operations are of greater magnitude, and the Brinton method is not dependable with castings weighing thirteen to twenty tons and upwards embodying sections of large surface area compared to their volume.

In practicing our invention, the casting is permitted to remain in the mould until it can be handled without bending, whereupon it is removed and the large surface areas 30 which disperse the heat rapidly are enveloped in a sand blanket. Thus protected, the casting is placed in a furnace which has been previously brought to a temperature of about 500° C. The furnace is immediately 35 sealed and held without firing in order to establish an even temperature of the furnace and casting. We maintain accurate pyrometer control, and when the reading indicates an even temperature we disperse the 40 heat slowly and uniformly, and, at a safe point, remove the sand blanket.

The casting denuded of sand is then heated slowly and uniformly, to the usual temperature for the treatment of manganese 45 steel, and is then quenched in water.

By our method of procedure we avoid the setting up of dangerous shrinkage stresses such as are prevalent when the castings are cooled below a red heat and during the 50 heating up of the castings from the mini-

mum temperature usually employed to a red heat.

Having described our invention, we claim:

1. The method of treating manganese steel 55 castings of large size and intricate form, which consists in blanketing the casting as soon as it can be handled without bending, and while so protected introducing it into a furnace previously heated to an annealing 60 temperature, sealing the furnace and controlling the heat so as to bring the furnace and casing to an even temperature, reducing the temperature slowly and uniformly to a predetermined point, removing the blanket, 65 and reheating slowly and uniformly to the usual temperature for the treatment of manganese steel, and then quenching in water.

2. The method of treating manganese steel 70 castings of large size and intricate form, which consists in sand protecting excessive heat dispersing sections as soon as the casting can be handled without bending, and while so protected introducing the casting into a furnace heated to about 500° C., sealing the furnace and holding it without firing until the furnace and the casting are at an even temperature, permitting the temperature to decline slowly and uniformly to a predetermined point, removing the 75 sand, raising the temperature at a slow and regulated rate to the usual temperature for the treatment of manganese steel, and rapidly quenching.

3. The method of treating manganese 85 steel castings of large size and intricate form, which consists in charging the casting, while hot from the casting heat, into a furnace heated to an annealing temperature, maintaining proper control to establish an 90 even temperature of the furnace and casting, gradually reducing the temperature to a predetermined point, and then slowly and uniformly heating the casting to the usual temperature for the treatment of manganese 95 steel, and quenching.

In testimony whereof we affix our signatures.

STANLEY APGAR.  
GEORGE R. HANKS.